

May 11, 1937.

A. A. WELLS

2,079,782

PROCESS OF DEODORIZING LUBRICATING OILS

Filed March 27, 1934



Alfred A. Wells Inventor

By W. E. Currie Attorney

## UNITED STATES PATENT OFFICE

2,079,782

## PROCESS OF DEODORIZING LUBRICATING OILS

Alfred A. Wells, Roselle Park, N. J., assignor to Standard Oil Development Company, a corporation of Delaware

Application March 27, 1934, Serial No. 717,541

2 Claims. (Cl. 196—29)

This invention relates to a process of producing lubricating oils of improved odor and will be understood from the following description when read in conjunction with the drawing the sole figure of which is a diagrammatic side elevation partly in section of an apparatus appropriate for carrying out the invention.

Lubricating oils which have been treated with an adsorbent clay often develop a disagreeable odor. This is especially the case with lubricating oils and cylinder stocks which have been finished by percolation through coarse clay such as coarse fuller's earth or Attapulgus clay. Such percolation is often carried out at temperatures ranging from 200—350° F. and higher. It is believed that this odor is caused by the action of the clay on the sulphur compounds, thereby forming H<sub>2</sub>S and similar compounds. I have found that the treatment of these oils with a small quantity of SO<sub>2</sub> in the presence of moisture will destroy this odor. The necessary time of treating can be shortened by raising the temperature to from 100° F. to 200° F. and above. A treating temperature of 150° F. very often gives good practical results. Any small excess of SO<sub>2</sub> can readily be removed by blowing with steam, air, inert gas, such as natural gas, refinery gas, nitrogen, CO<sub>2</sub>, etc., which at the same time brightens the oil due to the removal of the water vapors present.

Instead of using SO<sub>2</sub> gas, any compound such as, for example, sodium or potassium bi-sulphite, which contains a loosely bound SO<sub>2</sub> group can be used.

Referring now to the drawing, the same will be described in conjunction with the method of operating the apparatus shown. The lubricating oil from storage tank 1 is pumped through pre-heater 2 and percolating filter tank 3. The tank is filled with coarse clay 4 and provided with lagging 5 to prevent heat losses. The treated oil is then passed through heating or cooling coil 6 to adjust its temperature and is pumped into the deodorizing tank 7. When sodium bi-sulphite solution is used, the same may be pumped from the storage tank (not shown) through line 8 directly into the oil line leaving coil 6. Tank 7 is also provided with lagging 9 to prevent heat loss and with a steam or inert gas line 10 connected with line 11 for the introduction of SO<sub>2</sub>. The steam and SO<sub>2</sub> are discharged into tank 7 through the spray 12. The treated oil is removed through bottom line 13, cooler 14 into the finished oil tank 15. The steam and gas leave tank 7 through overhead line 16 and steam condenser 17. A receiver 18 for any condensate, vent line 19 and vacuum pump 20 are provided as shown.

The following examples will illustrate my invention: A cylinder oil which had been acid

treated and neutralized in the ordinary way was percolated through Attapulgus clay at a temperature of 250—300° F. The oil coming from the percolating unit was cooled to 150° F. and then blown with steam for a short period. SO<sub>2</sub> gas was then bubbled into the oil until a slight odor of SO<sub>2</sub> could be detected. The SO<sub>2</sub> supply was then shut off and the oil blown with air at 150° F. until the odor of SO<sub>2</sub> had disappeared. The disagreeable odor of the original percolated oil was largely removed.

In another experiment the sample of oil which had previously been percolated at a temperature above 250° F. and which had a disagreeable odor was heated to 150° F. while at the same time a small amount of steam was blown through the oil. A solution of sodium bi-sulphite was then added to the oil in the ratio of 0.35 gram of sodium bi-sulphite to a liter of oil and agitated with air for a brief period. The oil was then blown with steam at approximately 150° F. until the odor of sodium bi-sulphite had disappeared. The resulting oil was sweet in odor.

Still in another experiment the sample of oil which had been treated with SO<sub>2</sub>, as in the first example, was blown with nitrogen under a slight vacuum at a temperature of 200° F. to remove the traces of SO<sub>2</sub>. This sample had a particularly good odor.

In the following claims the term "lubricating oil" is meant to designate both lubricating oils and cylinder oils, whether obtained by overhead distillation or as residual stocks.

My process may be modified in various ways. The blowing with air or steam or inert gas may be carried out in atmospheric pressure or under vacuum. Other changes and modifications will be apparent to those skilled in the art. Therefore, my invention is not to be limited by the examples given for illustration but only by the following claims, in which it is my intention to claim all novelty inherent in the invention.

What I claim is:

1. An improved process for refining mineral lubricating oils and removing objectionable odors therefrom, comprising the separate steps of treating the oil with clay at a temperature of the order of 200° F. and higher, separating the clay and then agitating the oil with moist sulfur dioxide at a temperature below 200° F. and then removing any excess thereof.

2. A process according to claim 1 in which the clay treating step is accomplished at a temperature within the range from about 200° to 350° F., and treatment with moist sulfur dioxide at a lower temperature range within from about 100° to 200° F.

ALFRED A. WELLS.